



US006439002B1

(12) **United States Patent**  
**Driggs**

(10) **Patent No.:** **US 6,439,002 B1**  
(45) **Date of Patent:** **Aug. 27, 2002**

(54) **PRINT-RECEPTIVE, PILL-RESISTANT,  
KNITTED FLEECE FABRIC**

JP 48-61798 8/1973

**OTHER PUBLICATIONS**

(75) Inventor: **Sonny B. Driggs**, Advance, NC (US)

pp. 13-15 from Knitting Technology, 2<sup>nd</sup> Edition by David J. Spencer "A Comprehensive Handbook and Practical Guide to Modern Day Principles and Practices" First edition 1983.

(73) Assignee: **Sara Lee Corporation**, Winston-Salem, NC (US)

\* cited by examiner

(\*) Notice: Subject to any disclaimer, the term of this patent is extended or adjusted under 35 U.S.C. 154(b) by 0 days.

*Primary Examiner*—Andy Falik  
(74) *Attorney, Agent, or Firm*—Womble Carlyle Sandridge & Rice, PLLC

(21) Appl. No.: **09/798,325**

**ABSTRACT**

(22) Filed: **Mar. 2, 2001**

A print-receptive, pill-resistant, knitted fleece fabric and printed article of apparel. The fabric is knitted from yarn formed from high-tenacity, staple synthetic fiber having a tenacity value of greater than about 4 grams/denier and preferably about 6 grams/denier. The resulting knitted fleece fabric has a pilling resistance value of greater than about 3. In the preferred embodiment, the high-tenacity, staple synthetic fiber is selected from the group consisting of air jet spun polyester; nylon; acrylic; and polypropylene. The use of staple fibers improves the hand, drape and comfort of the knitted fabric. Also, in the preferred embodiment, the knitted fabric is a 3 end fleece fabric having a face yarn side and a lay-in yarn side, the face yarn side being formed from the high-tenacity, staple synthetic fiber and the lay-in yarn side being substantially formed from cellulosic yarns, such as cotton and synthetic cellulosic fibers or a synthetic/cellulosic blend. This construction improves both comfort and opacity of the knitted fabric while, at the same time, provides a print-receptive face and good print resolution of the article of apparel after multiple home washings.

**Related U.S. Application Data**

(63) Continuation-in-part of application No. 09/256,981, filed on Feb. 24, 1999, now Pat. No. 6,253,582.

(51) **Int. Cl.<sup>7</sup>** ..... **D04B 1/00**

(52) **U.S. Cl.** ..... **66/202**

(58) **Field of Search** ..... 66/202

(56) **References Cited**

**U.S. PATENT DOCUMENTS**

3,967,472 A \* 7/1976 Wildeman et al. ..... 66/191  
4,071,502 A \* 1/1978 Sugiyama et al. ..... 260/75 T  
5,038,584 A \* 8/1991 Wildeman ..... 66/192  
6,253,582 B1 \* 7/2001 Driggs ..... 66/202

**FOREIGN PATENT DOCUMENTS**

|    |         |         |
|----|---------|---------|
| DE | 2642350 | 3/1978  |
| FR | 2230794 | 12/1974 |
| GB | 1517832 | 7/1978  |

**24 Claims, 6 Drawing Sheets**





**FIG. 1**  
**PRIOR ART**



**FIG. 2**



**FIG. 3**



**FIG. 4**



**FIG. 5**



**FIG. 6**

PRINT-RECEPTIVE, PILL-RESISTANT,  
KNITTED FLEECE FABRICCROSS-REFERENCE TO RELATED  
APPLICATION

The present application is a continuation-in-part of U.S. patent application Ser. No. 09/256,981, filed Feb. 24, 1999 (now U.S. Pat. No. 6,253,582, issued Jul., 3, 2001).

## BACKGROUND OF THE INVENTION

## (1) Field of the Invention

The present invention relates generally to circular knitted fleece fabric and, more particularly, to a pill-resistant knitted fabric and article of apparel having a print-receptive face and good print resolution even after multiple home washings.

## (2) Description of the Prior Art

The term circular knitting covers those weft knitting machines having needle beds arranged in circular cylinders and/or dials including latch, bearded and occasionally compound needle machinery. Such machines produce a wide variety of fabric structures, garments, hosiery and other articles and a variety of diameters and machine gauges. Such machines have the needles fixed in a revolving circle with the loop formation and knitting action being achieved by ancillary elements moving yarn and loops along the needle stems producing a fabric tube with the technical face facing backwards. Large diameter circular knitting machines are generally used to produce either fleece or jersey fabrics as well as other fabric constructions. The following discussion is taken generally from Spencer, David J., *Knitting Technology*, (2d. ed. 1989), which is a general treatment of knitting technology and is hereby incorporated by reference in its entirety.

Knitted fabrics are progressively built up by converting newly fed yarn into new loops in the needle hooks, the needles then draw these new loops head first through the old loops, which have been retained from the previous knitting cycle. The needles at the same time release, cast off or knock-over old loops so that they hang suspended by their heads from the feet of the new loops whose heads are still held in the hooks of the needles. A cohesive structure is thus produced by a combination of the intermeshed loops and the yarn joining those loops together through which it passes.

Knitted loops are arranged in rows and columns roughly equivalent to the warp and weft of woven structures termed "courses" and "wales" respectively. A course is a predominately horizontal row of loops (in an upright fabric) produced by adjacent needles during the same knitting cycle. A wale is a predominantly vertical column of needle loops produced by the same needle knitting at successive knitting cycles and thus intermeshing each new loop through the previous loop.

"Yarn count" indicates the linear density (yarn diameter or fineness) to which that particular yarn has been spun. The choice of yarn count is restricted by the type of knitting machine employed and the knitting construction. The yarn count, in turn, influences the cost, weight, opacity, hand and drape of the resulting knitted structure. In general, staple spun yarns tend to be comparatively more expensive the finer their count, because finer fibers and a more exacting spinning process are necessary in order to prevent the yarn from showing an irregular appearance.

The conventional technique for painting or decorating fabrics, such as Tee shirts, is screen-printing. In a typical screen printing operation, a separate screen is made for each

color to be applied. A first screen is brought into registry with the fabric surface and a first color painted thereon. A second, third, and fourth screen, if necessary, each representing different colors, is then brought into registry with the surface and the additional colors painted or brushed thereon through the pattern in the screen.

In the textile industry, the problems associated with screen printing have been overcome, to some extent, by a process known as "heat-transfer printing" in which a carrier consisting usually of paper or aluminum foil is printed with sublimable dyes temporarily affixed to the carrier by the use of binders. The carrier so printed is then laid with the printed side adjacent the fabric to be printed, and is then heated under pressure to a temperature in the range of 160° C. to 220° C. on the unprinted side of the carrier to sublime the dyes onto the fabric.

Heat-transfer printing techniques have been attempted onto a wide variety of sheet-like articles such as wood, metals, glass, ceramics, and certain synthetic resins by providing such articles with a surface layer or coating of a thermoplastic resin which adheres to the surface of the substrate and accepts the sublimable dyes. See e.g., German patent No. DE 2,642,350; French Pat. No. 2,230,794; and British Pat. No. 1,517,832. Similarly, the surface of the article to be printed may be coated with a thermosetting resin (published European patent application No.14,901) which receives the dyes. Characteristic of all of the above approaches is that the transfer of the dyes by sublimation onto a thermosetting or thermoplastic resin is effected by means of heat supplied or generated by an external source.

Natural fibers, such as cotton and rayon, do not readily accept or retain sublimable dyes. Because of this shortcoming, polyester/cotton blends dyed in this way exhibit "grin through" since the cotton portion of the fabric remains undyed. In addition, polyester/ cotton blends are notorious for "pilling" which further degrades the printed image after a few home washings. While it is generally believed that pilling only occurs with polyester/cotton blends, pilling will also occur in knitted 100% polyester fabrics if staple yarns are used. However, this is not usually observed since polyester staple fibers are seldom used without first being blended with cotton fibers because 100% polyester fabric is uncomfortable to wear against the skin. Consequently, most 100% polyester fabrics that are used for apparel are usually either knitted or woven continuous multi-filament yarns because of the high strength and low cost of these yarns.

Woven 100% synthetic fabric is an ideal substrate for receiving sublimable dyes because of the composition of the yarn and the stability of a woven construction. Unfortunately, the hand, drape, opacity and comfort of a woven 100% polyester fabric are even more unacceptable to the average consumer than the poor appearance of "grin through". As a result, 100% polyester sublimable dyed woven fabrics are usually reserved for banners and other non-apparel uses.

Thus, there remains a need for a new and improved fleece fabric that is print receptive to sublimable dyes like a 100% synthetic fabric and pill-resistant like a continuous multi-filament synthetic fabric while, at the same time, provides the comfort and appearance of a knitted cotton or cotton/polyester stable blend which is suitable for apparel articles, such as Tee shirts.

## SUMMARY OF THE INVENTION

The present invention is directed to a print-receptive, pill-resistant, knitted fleece fabric. The fabric is knitted from

yarn formed from high-tenacity, staple synthetic fiber having a tenacity value of greater than about 4 grams/denier and preferably about 6 grams/denier. Surprisingly, the resulting knitted fleece fabric has a pilling resistance value of greater than about 3. In the preferred embodiment, the high-tenacity, staple synthetic fiber is selected from the group consisting of air jet spun polyester nylon; acrylic; and polypropylene. The use of staple fibers improves the hand, drape and comfort of the knitted fabric. Also, in the preferred embodiment, the knitted fleece fabric is a three-end fleece fabric having a face yarn side and a lay-in yarn side (sometimes called the backing yarn), the face yarn side being formed from the high-tenacity, staple synthetic fiber and the lay-in yarn side being substantially formed from cellulosic yarns, such as cotton and rayon. This construction improves both comfort and opacity of the knitted fabric while, at the same time, provides a print-receptive, pill-resistant face.

Accordingly, one aspect of the present invention is to provide a print-receptive, pill-resistant, knitted fleece fabric. The fabric is knitted from yarn formed from high-tenacity, staple synthetic fiber having a tenacity value of greater than about 4 grams/denier, wherein the knitted fleece fabric has a pilling resistance value of greater than about 3.

Another aspect of the present invention is to provide a print-receptive, pill-resistant, knitted fleece fabric. The fabric is knitted from yarn formed from high-tenacity, staple synthetic fiber having a tenacity value of greater than about 4 grams/denier, wherein the knitted fleece fabric has a pilling resistance value of greater than about 3, and the high-tenacity, staple synthetic fiber is selected from the group consisting of air jet spun polyester; nylon; acrylic; and polypropylene.

Still another aspect of the present invention is to provide a print-receptive, pill-resistant, knitted fleece fabric. The fabric is knitted from yarn formed from high-tenacity, staple synthetic fiber having a tenacity value of greater than about 4 grams/denier, wherein the knitted fleece fabric has a pilling resistance value of greater than about 3, and the high-tenacity, staple synthetic fiber is selected from the group consisting of air jet spun polyester; nylon; acrylic; and polypropylene, and wherein the knitted fleece fabric is a three-end fleece fabric having a face yarn side and a lay-in yarn side, the face yarn side being substantially formed from the high-tenacity, staple synthetic yarn and the lay-in yarn side being substantially formed from the cellulosic yarn, the cellulosic yarn being selected from the group consisting of cotton and rayon fibers.

#### BRIEF DESCRIPTION OF THE DRAWINGS

FIG. 1 is a photomicrograph of a conventional jersey cotton knitted fabric, normally used for Tee shirts, illustrating its construction and cover;

FIG. 2 is a photomicrograph of a double knit fabric, constructed according to the parent invention, illustrating its construction and similar cover;

FIG. 3 is a cross-sectional view of the double knit fabric of the parent invention shown in FIG. 2;

FIG. 4 is a photomicrograph of the face of a knitted fleece fabric, constructed according to the present invention, illustrating its construction;

FIG. 5 is a photomicrograph of the napped back of the knitted fleece fabric shown in FIG. 4, illustrating its construction; and

FIG. 6 is a cross-sectional view of the knitted fleece fabric shown in FIG. 4.

#### DESCRIPTION OF THE PREFERRED EMBODIMENTS

In the following description, like reference characters designate like or corresponding parts throughout the several views. Also in the following description, it is to be understood that such terms as "forward", "rearward", "left", "right", "upwardly", "downwardly", and the like are words of convenience and are not to be construed as limiting terms.

The parent invention can be practiced using a conventional or a convertible circular knitting machine, such as set forth in the U.S. Pat. No. 5,613,375, which is hereby incorporated by reference in its entirety. The knitting machine includes four major sub-assemblies: a creel having a plurality of yarn packages; a plurality of feeders; a knitting cylinder supported on a bed and having a plurality of needles; and a plurality of section blocks attached to the bed and arranged about the perimeter of the cylinder.

Jersey fabric is usually knit on four feeds per block. Only one yarn is necessary to knit a course of jersey fabric. Accordingly, one cam and one yarn will knit one course of jersey fabric. Three cams in each block would make three courses of jersey fabric. Three times 36 jersey section blocks would make 108 courses per cylinder revolution. The more cams around the circumference, the more production. An example of such a fabric is shown in FIG. 1.

According to the parent invention, fabrics were formed from a variety of yarns into a double knitted jersey fabric. The face of each jersey fabric was a synthetic yarn, such as polyester, nylon, acrylic or polypropylene. The back of each jersey fabric was a cellulosic fiber, such as cotton. An example of this double-knit jersey fabric is shown in FIG. 2. A cross-sectional view of the double knit jersey fabric shown in FIG. 2 is shown in FIG. 3.

The knitted construction of the parent invention was generally conventional and was knitted on an eight lock double knit machine having a two track cylinder and a two track dial. This arrangement provides the versatility to knit, tuck and float on all feeds. In the most preferred embodiment, the knitting machine was set up such that the fabric layer knit on the cylinder was either 100% synthetic yarn or 100% cellulosic (e.g. cotton and other natural plant fibers, rayon, acetate and triacetate) and the fabric layer on the dial being the opposite yarn. The resulting jersey fabric was an outer layer of print receptive synthetic yarn and an inner layer of cellulosic yarn. As can be appreciated, the cellulosic yarn layer could be 100% cotton or a blend of cotton/polyester.

After formation, each jersey fabric sample was printed with a sublimable dye and tested for print resolution before and after a 15 home wash and dry laundering wash test using a 1-5 scale with 5 being best. The samples were also evaluated for hand, drape, opacity and comfort on a similar scale. Finally, each sample was tested for pilling resistance using the Random Tumble Pilling test procedure. The results can best be understood by referring to Table 1 below:

TABLE 1

| Fabric Construction                                                                                | Print Resolution (before & after 15 washings) |       |         |         |    |    | Pilling Resistance* (with & wo cotton fibers) |   |
|----------------------------------------------------------------------------------------------------|-----------------------------------------------|-------|---------|---------|----|----|-----------------------------------------------|---|
|                                                                                                    | Hand                                          | Drape | Opacity | Comfort |    |    |                                               |   |
| 100% ring spun polyester (Example 1)                                                               | 5                                             | 3.5   | 1       | 1       | 1  | 1  | 2.5                                           | — |
| 100% polyester Comfortrel® (Example 2)                                                             | 5                                             | 3     | 4       | 1       | 2  | 3  | 2                                             | — |
| Plating poly to face and cotton to back (Example 3)                                                | 3 (grin thru)                                 | 2     | 4       | 4       | 4  | 3  | 2.5                                           | — |
| Double-knit with ploy to face and cotton to back (Example 4)                                       | 5                                             | 3.5   | 3       | 4       | 4+ | 4- | 2.5                                           | 2 |
| Double-knit w/ Comfortrel® to face and cotton to back (Example 5)                                  | 5                                             | 3.5   | 4       | 4       | 4+ | 4+ | 2.5                                           | 3 |
| Double-knit with high tenacity, air jet spun polyester yarn to face and cotton to back (Example 6) | 5                                             | 5     | 4       | 4       | 4+ | 4+ | 3.0                                           | 4 |

\*pilling resistance was tested according to ASTM D3512-82 test method both with and without the introduction of cotton fibers into the test chamber.

30

As can be seen, 100% polyester jersey fabric had good print resolution after washing but poor hand, drape, opacity and comfort. Surprisingly, its pilling resistance was only average. Substituting Comfortrel®, variable staple length fibers improved hand, opacity and comfort but, surprisingly, did not help drape or pilling resistance.

As can also be seen, plating the polyester with cotton did improve hand, drape, opacity and comfort but “grin through” and pilling resistance were only average. In addition, the plating process was hard to control and, as a result, the placement of the yarns varied.

The double knitted, jersey fabric of the parent invention (examples 4–6) produced very good print resolution after washing with high hand, drape, opacity and comfort values. In addition, the use of Comfortrel® fibers (example 5) further improved the hand but, surprisingly, did not improve the pilling resistance of the polyester face.

However, surprisingly, the use of higher tenacity yarns (example 6) substantially eliminated that shortcoming while, at the same time, maintained the other critical values of print resolution after washing, hand, drape, opacity and comfort. The original Comfortrel® fibers had a tenacity of about 3 grams/denier. The higher tenacity yarns (example 6) had a tenacity of about 6 grams/denier and, unexpectedly, did not pill. This is contrary to the generally accepted idea of reducing the tenacity of the synthetic yarns when pilling occurs to allow the pills to more easily break off.

In the most preferred embodiment, shown in example 6, the high-tenacity, staple synthetic fiber is polyester having a denier of less than about 1.5 and preferably about 1. Also, the staple length of this high-tenacity, synthetic fiber was about 1.5 inches but variable lengths up to about 1.5 inches would be expected to work as well. The above data illustrates that a knitted jersey fabric constructed according to the parent invention is print receptive and pill resistant, thereby providing excellent print resolution even after 15 home washings.

An article of apparel formed from the jersey fabric of the parent invention may be printed using, for example, a Sawgrass Sublijet ink system in an Epson 3000 ink jet printer and transferring the image to the polyester print receptive surface. Preferably, the image is composed using conventional desktop publishing software, such as Hanes T-ShirtMaker, and printed on high-quality ink jet transfer paper, such as “ColorTrans” paper from Wyndstone. The actual transfer to the apparel may be done using an Insta-Graphic beat press set at about 400 degrees F and pressing for about 20 seconds.

The present invention, which is a printable, pill resistant, three-end fleece fabric, also can be practiced using a conventional or a convertible circular knitting machine, such as set forth in the U.S. Pat. No. 5,613,375, which is hereby incorporated by reference in its entirety. The knitting machine includes four major sub-assemblies: a creel having a plurality of yarn packages; a plurality of feeders; a knitting cylinder supported on a bed and having a plurality of needles; and a plurality of section blocks attached to the bed and arranged about the perimeter of the cylinder.

Fleece fabric is usually knit on three feeds per block. According to the present invention, fabrics were formed from a variety of yarns into a three-end, fleece fabric. The face yarn of each three-end, fleece fabric was a synthetic yarn, such as polyester, nylon, acrylic or polypropylene. The lay-in yarn of each three-end, fleece fabric was substantially a cellulosic fiber, such as cotton, and is preferably, a blend of 50% cotton and 50% polyester. The filler yarn was also a synthetic yarn, such as polyester, nylon, acrylic or polypropylene. An example of this three-end, fleece fabric is shown in FIGS. 4 and 5. A cross-sectional view of the three-end, fleece fabric shown in FIG. 6.

The knitted construction of the present invention was generally conventional and was knitted on a 3 end fleece machine having a four track cylinder. This arrangement

35

40

45

50

55

60

65

provides the versatility of different lay-in pattern constructions. In the most preferred embodiment, the knitting machine was set up such that the jersey face and filler yarns knit on the cylinder were 100% synthetic yarn and the lay-in interface yarn was 50/50 synthetic and cotton. The resulting fabric was an outer layer of print receptive synthetic yarn and an inner layer of a sufficient amount of cellulosic yarn for comfort. As can be appreciated, the lay-in interface yarn could be 100% cotton where more comfort is desired or a 100% polyester where it is not needed. When 100% cotton is used for the lay-in yarn, the fabric would not be napped

After formation, each three-end, fleece fabric sample was printed with a sublimable dye and tested for print resolution before and after a 15 home wash and dry laundering wash test using a 1-5 scale with 5 being best. The samples were also evaluated for hand, drape, cover and comfort on a similar scale. Finally, each sample was tested for pilling resistance using the Random Tumble Pilling test procedure. The results can best be understood by referring to Table 2 below:

TABLE 2

| Fabric Construction                                                                                                                      | Print Resolution (before & after 15 washings) |       |       |         | Pilling Resistance* (with & w/o cotton fibers) |    |     |   |
|------------------------------------------------------------------------------------------------------------------------------------------|-----------------------------------------------|-------|-------|---------|------------------------------------------------|----|-----|---|
|                                                                                                                                          | Hand                                          | Drape | Cover | Comfort |                                                |    |     |   |
| 3 end fleece 100% spun polyester on face, filler and lay-in (Example 1)                                                                  | 5                                             | 4     | 3     | 3.5     | 3                                              | 3  | 2.0 | — |
| 3 end fleece with poly to face and filler and poly/cotton to lay-in (Example 2)                                                          | 5                                             | 3.5   | 3.5   | 3.5     | 3                                              | 4- | 2.5 | 2 |
| 3 end fleece w/ Comfortrel® to face and filler and poly/cotton to lay-in (Example 3)                                                     | 5                                             | 3.5   | 4     | 4       | 3                                              | 4+ | 2.5 | 3 |
| 3 end fleece with high tenacity, air jet spun polyester yarn to face, textured polyester to filler and poly/cotton to lay-in (Example 4) | 5                                             | 5     | 4     | 4       | 4+                                             | 4+ | 3.0 | 4 |

\*pilling resistance was tested according to ASTM D3512-82 test method both with and without the introduction of cotton fibers into the test chamber.

because 100% napped cotton can be more susceptible to ignition. However, the face of the fabric would still be print receptive.

Thus, the present 3 end fabric includes a face yarn, a filler 50 yarn that rides with the face yarn and a lay-in yarn. In the preferred embodiment, the face yarn is an air jet spun 100% polyester yarn, the filler yarn is a textured 100% polyester yarn and the lay-in yarn is a 50/50 polyester/cotton blend. However, as mentioned above, in an alternative embodiment, both the face and the filler yarns could be an air jet spun 100% polyester yarn and the lay-in yarn could be a 100% spun polyester.

As, as will be further discussed below, the textured 100% polyester filler yarn provided better cover of the lay-in yarn and, therefore, better print performance while, at the same time, was less expensive than air jet spun 100% polyester yarn. In addition, the improvement in cover also allowed the use of the 50/50 polyester/cotton blend for the lay-in yarn, which is generally less expensive than a 100% spun polyester yarn. Finally, the 50/50 polyester/cotton lay-in yarn was more easily napped than a 100% spun polyester yarn.

As can be seen, the 100% polyester three-end, fleece fabric in Example 1 had good print resolution after washing but less desirable hand, drape, cover and comfort. Surprisingly, its pilling resistance was only average. Substituting polyester/cotton lay-in in Example 2 improved hand and comfort but did not help cover or pilling resistance.

As can also be seen, substituting Comfortrel® variable staple length polyester fibers and polyester/cotton lay-in in Example 3 did improve hand, drape and comfort but cover and pilling resistance were only average.

To the contrary, the three end fleece fabric of the present invention (example 4) produced very good print resolution after washing with high hand, drape and comfort values.

Moreover, surprisingly, the use of higher tenacity yarns on the face and textured polyester yarn in the filler substantially eliminated the cover and pilling shortcomings while, at the same time, maintained the other critical values. The original Comfortrel® fibers had a tenacity of about 3 grams/denier. The higher tenacity yarns (example 4) had a tenacity of about 6 grams/denier and, unexpectedly, did not pill. This is contrary to the generally accepted idea of reducing the

tenacity of the synthetic yarns when pilling occurs to allow the pills to more easily break off.

In the most preferred embodiment, shown in example 4, the high-tenacity, staple synthetic fiber is polyester having a denier of less than about 1.5 and preferably about 1. Also, the staple length of this high-tenacity, synthetic fiber was about 1.5 inches but variable lengths up to about 1.5 inches would be expected to work as well. The above data illustrates that a knitted fabric constructed according to the present invention is print receptive and pill resistant, thereby providing excellent print resolution even after 15 home washings.

An article of apparel formed from the fabric of the present invention may be printed using, for example, a Sawgrass Sublijet ink system in an Epson 3000 ink jet printer and transferring the image to the polyester print receptive surface. Preferably, the image is composed using conventional desktop publishing software, such as Hanes T-ShirtMaker, and printed on high-quality ink jet transfer paper, such as "ColorTrans" paper from Wyndstone. The actual transfer to the apparel may be done using an Insta-Graphic heat press set at about 400 degrees F. and pressing for about 20 seconds.

Certain modifications and improvements will occur to those skilled in the art upon a reading of the foregoing description. By way of example, a substantially 100% cellulosic layer could be used instead of a blend of natural and synthetic fibers for particular applications and markets. Similarly, the substantially 100% polyester layer could be altered to include other synthetic fibers for particular applications and markets. Also, finishes may be applied to the fabric either during knitting or afterwards to further improve desirable fabric characteristics, such as shown in Table 2. It should be understood that all such modifications and improvements have been deleted herein for the sake of conciseness and readability but are properly within the scope of the following claims.

I claim:

1. A print-receptive, pill-resistant, knitted fleece fabric, said fabric knitted from yarn formed from high-tenacity, staple synthetic fiber wherein the high-tenacity, staple synthetic fiber has a tenacity of about 6 grams/denier, and wherein said knitted fleece fabric has a pilling resistance value of greater than about 3.

2. The knitted fabric of claim 1, wherein said knitted fleece fabric is a fabric having a face yarn side and a lay-in yarn side, the face yarn side being formed from said high-tenacity, staple synthetic fiber and the lay-in yarn side being substantially formed from cellulosic yarn, said cellulosic yarn being selected from the group consisting of cotton and synthetic cellulosic fibers.

3. The knitted fabric of claim 1, wherein the lay-in yarn side of said fabric is substantially 50/50% spun cotton/polyester fiber.

4. The knitted fabric of claim 1, wherein the face yarn side and lay-in yarn side of said fabric are a three-end fleece knit construction.

5. The knitted fabric of claim 1, further including a filler yarn between the face yarn and lay-in yarn of said fabric.

6. A print-receptive, pill-resistant, knitted fleece fabric, said fabric knitted from yarn formed from high-tenacity, staple synthetic fiber having a tenacity value of greater than about 4 grams/denier, wherein said knitted fleece fabric has a pilling resistance value of greater than about 3, and said high-tenacity, staple synthetic fiber is selected from the group consisting of air jet spun polyester; nylon; acrylic; and polypropylene.

7. The knitted fabric of claim 6, wherein said high-tenacity, staple synthetic fiber is polyester.

8. The knitted fabric of claim 6, wherein said high-tenacity, staple synthetic fiber has a denier of less than about 1.5.

9. The knitted fabric of claim 8, wherein said high-tenacity, staple synthetic fiber has a denier of about 1.

10. The knitted fabric of claim 6, wherein the staple length of said high-tenacity, synthetic fiber is about 1.5 inches.

11. The knitted fabric of claim 10, wherein the staple length of said high-tenacity, synthetic fiber is variable up to about 1.5 inches.

12. A print-receptive, pill-resistant, knitted fleece fabric, said fabric knitted from yarn formed from high-tenacity, staple synthetic fiber having a tenacity value of greater than about 4 grams/denier, wherein said knitted fleece fabric has a pilling resistance value of greater than about 3, and said high-tenacity, staple synthetic fiber is selected from the group consisting of air jet spun polyester; nylon; acrylic; and polypropylene, and wherein said knitted fabric is a fabric having a face yarn side and a lay-in yarn side, the face yarn side being formed from said high-tenacity, staple synthetic fiber and the lay-in yarn side being substantially formed from cellulosic yarn, said cellulosic yarn being selected from the group consisting of cotton and synthetic cellulosic fibers.

13. The knitted fabric of claim 12, wherein the lay-in yarn side of said fabric is substantially 50/50% spun cotton/polyester fiber.

14. The knitted fabric of claim 12, wherein the face yarn side and lay-in yarn side of said fabric are a three-end fleece knit construction.

15. The knitted fabric of claim 12, further including a filler yarn between the face yarn and lay-in yarn of said fabric.

16. The knitted fabric of claim 12, wherein the high-tenacity, staple synthetic fiber has a tenacity of about 6 grams/denier.

17. The knitted fabric of claim 12, wherein said high-tenacity, staple synthetic fiber is polyester.

18. The knitted fabric of claim 12, wherein said high-tenacity, staple synthetic fiber has a denier of less than about 1.5.

19. The knitted fabric of claim 18, wherein said high-tenacity, staple synthetic fiber has a denier of about 1.

20. The knitted fabric of claim 12, wherein the staple length of said high-tenacity, synthetic fiber is about 1.5 inches.

21. The knitted fabric of claim 20 wherein the staple length of said high-tenacity, synthetic fiber is variable up to about 1.5 inches.

22. A printed, pill-resistant, article of fleece apparel, said article of apparel knitted from yarn formed from high-tenacity, staple synthetic fiber having a tenacity value of greater than about 4 grams/denier, wherein said article of apparel has a pilling resistance value of greater than about 3.

23. A printed, pill-resistant, article of fleece apparel, said article of apparel knitted from yarn formed from high-tenacity, staple synthetic fiber having a tenacity value of greater than about 4 grams/denier, wherein said article of apparel has a pilling resistance value of greater than about 3, and said high-tenacity, staple synthetic fiber is selected from the group consisting of air jet spun polyester; nylon; acrylic; and polypropylene.

24. A printed, pill-resistant, article of fleece apparel, said article of apparel knitted from yarn formed from high-tenacity, staple synthetic fiber having a tenacity value of greater than about 4 grams/denier, wherein said article of apparel

apparel has a pilling resistance value of greater than about 3, and said high-tenacity, staple synthetic fiber is selected from the group consisting of air jet spun polyester; nylon; acrylic; and polypropylene, and wherein said article of apparel is formed from a fabric having a face yarn side and a lay-in 5 yarn side, the face yarn side being formed from said high-

tenacity, staple synthetic fiber and the lay-in yarn side being substantially formed from cellulosic yarn, said cellulosic yarn being selected from the group consisting of cotton and synthetic cellulosic fibers.

\* \* \* \* \*